

Patented Aug. 26, 1930

1,773,975

# UNITED STATES PATENT OFFICE

GEORGE HOLLAND ELLIS AND RALPH JAMES MANN, OF SPONDON, NEAR DERBY, ENGLAND, ASSIGNORS TO CELANESE CORPORATION OF AMERICA, A CORPORATION OF DELAWARE

## PRODUCTION OF NEW OR IMPROVED FABRICS OR ARTICLES

No Drawing. Application filed May 17, 1927, Serial No. 192,159, and in Great Britain June 15, 1926.

This invention relates to the production of effects or patterns on woven, knitted or other textile fabrics or articles made from or containing cellulose acetate threads or yarns.

- 5 According to the present invention we have found that excellent patterns or effects constituted by local difference of lustre may be produced upon woven, knitted, or other textile fabrics or articles made from or containing cellulose acetate threads or yarns by the local application to said fabrics or articles of one or more of the following substances, and by subsequently subjecting the fabrics or articles to the delustering action of 10 steam or other hot or boiling aqueous media. The substances we employ for the local application according to the present invention are mono or poly basic carboxylic acids of the aliphatic series and substituted derivatives 15 thereof such as halogen derivatives, amino derivatives, hydroxy derivatives; the hydroxy derivatives being especially advantageous.

As examples of such bodies may be mentioned:—formic, acetic, propionic, butyric, chloracetic, aminoacetic, glycollic, lactic, citric, succinic acids, but it is of course understood that we in nowise limit ourselves to these examples.

The local application may be performed by 30 any suitable means such for instance as printing, stencilling and the like, and may be applied to form any suitable desired pattern, for instance a figured design or pattern or a ground or "blotch" which leaves a figured 35 design or pattern in relief.

After the local application we subject the goods to the delustering treatment preferably by subjecting them to the action of steam.

Under given conditions of steaming some 40 of these agents are found to act in a protective way, that is to say, they retard the rate at which cellulose acetate loses its lustre in the steam, whilst others act in the opposite way. By use of chosen agents at suitable concentrations it is possible to decrease or accel-

erate the rate of loss of lustre to such an extent as compared with the normal that the lustre of the one portion may be practically unchanged whilst that of the other portion is so modified as to enable very distinct, sharp 50 and clear patterns to be executed. The effects in many cases are quite permanent and will withstand treatment in the laundry as well as ordinary domestic usage. The cellulose acetate materials can of course be already dyed 55 by known methods before application of the process according to this invention, which process is found not to disturb or affect the dyeings. Alternatively it is found satisfactory to dye the materials subsequent to the 60 process. Mixed materials of cellulose acetate and other textile fibres may be similarly treated when the lustre of the former only is substantially affected so that a wide field 65 of possible effects is opened up by use of such materials. Furthermore, as is well known, such materials are capable of yielding differential colorings by the employment of appropriate coloring matters for the different components, which again adds to the 70 great variety of effects producible.

In carrying out the process where the agent to be applied locally is soluble in water, it will usually be applied from aqueous solution. Where it is less soluble, insufficiently 75 soluble or insoluble, it may be applied either in suspension with or without protective colloids, or dispersed by any known or suitable means such for example as the so called colloidal milling or by physical methods such 80 for example as forming dispersions with the aid of known emulsifying or dispersing agents, or by dissolving the agents of the present invention in organic solvents and pouring the solution into or diluting it with 85 water in presence or absence of protective colloids. For applying by the usual methods of printing such solutions or dispersions will usually be thickened by appropriate known substances such as starches, gums, flours and 90

the like, or for stencilling they may be applied in the form of a spray with little or no thickening. After printing or other selected mode of application the goods are preferably dried and then subjected to the action of steam in a suitable apparatus such as the familiar "ager", "cottage" or "continuous steamer" common in the textile printing industries, until the required effect or differential lustre is produced. The goods may then be rinsed to remove thickening and residual agent and further washed and finished as desired or requisite. While we preferably subject the goods to steaming after the local application it is of course to be understood that we may employ hot or boiling water, soap solutions, solutions of acids, or solutions of acid salts instead of steam.

The following examples serve to illustrate how the present invention may be performed, it being understood that they are in no way limitative.

#### Example 1

Print a knitted fabric composed of cellulose acetate yarns with the following paste:—  
 25 25 parts by weight succinic acid  
 70 70 parts by weight wheat starch thickening (15%)  
 30 5 parts by weight sodium sulpho ricinoleate (100%) or the equivalent amount of commercial Turkey red oil.  
 100

35 the acid and water are mixed together and added to the starch paste at 80° C. till dissolved. The paste is then cooled and suitably strained.

After printing, the fabric is dried quickly 40 and steamed in moist steam for 5 minutes after which it may be rinsed, soaped, dried and finished as desired or requisite. The printed portions in this case will have lost practically all their lustre and the unprinted portions remain substantially unchanged. 45 The pattern will therefore be chosen accordingly.

#### Example 2

Print a knitted fabric composed of cellulose acetate yarns, with the following paste:—  
 50 20-25 parts citric acid  
 70 70 parts wheat starch thickening (15%)  
 55 10-5 parts water  
 100

60 The acid and water are mixed together and added to the starch paste at 80° C. till dissolved. The paste is then cooled and suitably strained.

After printing the fabric is dried quickly and steamed in moist steam for 5 minutes after which it may be rinsed, soaped, dried and finished as desired or requisite. The

printed portions in this case will have lost practically all their lustre and the unprinted portions remain substantially unchanged. The pattern will therefore be chosen accordingly.

70

#### Example 3

For protection print with:—

10-30 parts acetic acid  
 70 parts wheat starch thickening (15%)  
 20-0 parts water  
 100

75

Steam until differences of lustre are sufficiently accentuated. In this case the printed portions will substantially have retained their original lustre and the unprinted portions become delustered. The pattern will therefore be chosen accordingly. After the steaming the fabrics may be rinsed, soaped, dried and finished as desired or requisite.

80

#### Example 4

For protection print with:—

10-30 parts chlor-acetic acid  
 70 parts wheat starch thickening (15%)  
 20-0 parts water  
 100

90

Steam until differences of lustre are sufficiently accentuated. In this case the printed portions will substantially have retained their original lustre and the unprinted portions become delustered. The pattern will therefore be chosen accordingly. After the steaming the fabrics may be rinsed, soaped, dried and finished as desired or requisite.

100

105

#### Example 5

For protection print with:—

10-30 parts propionic acid  
 70 parts wheat starch thickening (15%)  
 20-0 parts water  
 100

110

Steam until differences of lustre are sufficiently accentuated. In this case the printed portions will substantially have retained their original lustre and the unprinted portions become delustered. The pattern will therefore be chosen accordingly. After the steaming the fabrics may be rinsed, soaped, dried and finished as desired or requisite.

115

What we claim and desire to secure by Letters Patent is:—

1. Process for production of pattern effects on materials comprising cellulose acetate, comprising locally applying to the materials aliphatic carboxylic acids and thereafter delustering with hot aqueous media.

120

125

130

2. Process for production of pattern effects on materials comprising cellulose acetate, comprising locally applying to the materials aliphatic carboxylic acids and thereafter delustering with moist steam.
  3. Process for production of pattern effects on materials comprising cellulose acetate, comprising locally applying to the materials substituted aliphatic carboxylic acids and thereafter delustering with hot aqueous media.
  4. Process for production of pattern effects on materials comprising cellulose acetate, comprising locally applying to the materials substituted aliphatic carboxylic acids and thereafter delustering with moist steam.
  5. Process for the production of pattern effects on materials comprising cellulose acetate, comprising printing the materials with pastes comprising aliphatic carboxylic acids and thereafter delustering with moist steam.
  6. Process for the production of pattern effects on materials comprising cellulose acetate, comprising printing the materials with pastes comprising aliphatic carboxylic acids and thereafter delustering with moist steam.
  7. Process for the production of pattern effects on materials comprising cellulose acetate, comprising printing the materials with pastes comprising aliphatic carboxylic acids, drying and thereafter delustering with moist steam.
  8. Process for the production of pattern effects on materials comprising cellulose acetate, comprising printing the materials with pastes comprising substituted aliphatic carboxylic acids, drying and thereafter delustering with moist steam.
- 40 In testimony whereof we have hereunto subscribed our names.

GEORGE HOLLAND ELLIS.  
RALPH JAMES MANN.

45

50

55

60

65